# EUROPEAN PATENT APPLICATION

(11) **EP 2 881 002 A1**
(43) Date of publication of application: **10.06.2015**
(21) Application number: 13005702.9
(22) Date of filing: 06.12.2013
(51) Int. Cl.: A24B 15/20, A24B 3/18

(54) **Methods, uses and apparatus for increasing the filling power of tobacco**

(71) Applicant: Philip Morris Products S.A., 2000 Neuchâtel (CH)
(72) Inventor: Buehler, Frédéric Ulysse, 2000 Neuchâtel (CH)
(74) Representative: Grünecker Patent- und Rechtsanwälte PartG mbB

(57) **Abstract**

The invention relates to methods, uses and an apparatus for increasing the filling power of tobacco. These methods, uses and apparatus employ one or more enzymes capable of partially degrading cell walls of tobacco to unlock mechanical constraints prior to drying.

## Description

The present invention relates to methods, uses and an apparatus for increasing the filling power of tobacco by utilizing one or more enzymes to unlock the mechanical constraints of the cell walls in the tobacco. The invention further relates to a method of subjecting the tobacco treated with the one or more enzymes to a drying process.

In the tobacco industry, increasing the filling power of tobacco may be desired. In the prior art, it is known to expand tobacco for the purpose of improving its filling properties. A majority of known methods comprise placing wet cut tobacco into a high velocity and high temperature air flow to dry and expand the tobacco at the same time. The expansion of the tobacco is directly related to the rapid increase of the temperature. This is due to the changes in the cell structure of the tobacco being exposed to high temperatures within a very short period. The mechanism of expansion relies on the phase change of an expansion medium in the tobacco from liquid to vapor. Further, the speed at which this phase change occurs is critical to the level of expansion.

Current methods of expansion can be divided into two categories. In the first category, the tobacco is impregnated with an expansion agent, such as carbon dioxide for dried ice expanded tobacco or liquid nitrogen for inert gas compression. In the second category, water found in the cells of the tobacco is used as the expansion medium. The first category provides good expansion of the tobacco, but it requires the additional impregnation process to allow the expansion agents to permeate the tobacco cells. This method of expansion is extremely costly due to the increase of infrastructure required to build and house the capital equipment necessary to process the tobacco. The second category provides some expansion, but it has reduced effectiveness due to the limitations placed on the maximum temperature and duration which the increased temperature can be applied to the tobacco. If a high temperature is used, or a temperature is applied to the tobacco for too long, there can be an undesired impact on taste or quality of the expanded tobacco.

Therefore, there is a need for an improved method and means for increasing the filling power of tobacco which are more effective than current methods.

It is one object of the present invention to provide a new and improved method and means for increasing the filling power of tobacco. It is an additional object of the present invention to provide a method and means for enhancing the filling power of tobacco by subjecting the treated tobacco to a drying process.

The present invention enhances the filling power of tobacco by utilizing one or more enzymes to unlock mechanical constraints of intact tobacco cell walls and subjecting the treated tobacco to a drying process. The one or more enzymes are used to partially degrade cell walls of the tobacco to enable the tobacco to be expanded through drying. It is important that the cells walls of the tobacco are only partially degraded as full degradation of the cell walls will produce a tobacco which will be unsuitable for expansion. It is equally important, however, that there is degradation of the cell walls enough to enable expansion of the tobacco and increase the filling power of the tobacco material.

The present invention provides a method of partially degrading the cell walls of tobacco material, the method comprising the steps of:
a) contacting the tobacco material with an aqueous solution of one or more enzymes;
b) incubating the tobacco material with the aqueous solution of one of more enzymes for a period of 1 to 20 hours; and
c) drying the enzyme-treated tobacco material.

Preferably the one or more enzymes are capable of degrading cellulose and suitable for use in the present invention. The enzymes capable of degrading cellulose are found in the cellulase enzyme complex and include cellubiases, endocellulases, and exocellulases. Other enzymes include proteases, pectinases, polygalacturonases, cellulose 1,4-beta-cellobiosidases, endogluconases, endogluconase II, exo-cellubiohydolases, cellobiohydrolases, and cellobiases. Preferred enzymes are endogluconases, cellulases, and proteases.

Cellulases are an enzyme complex which breaks down cellulose to beta-glucase, depending on the length of time the tobacco is mixed with the cellulase. Cellulases often refers to a family of enzymes which act to hydrolyze cellulose. Typically, three general types of enzymes make up the cellulase enzyme complex. The first, endocellulases, breaks internal bonds to disrupt the crystalline structure of cellulose and expose individual cellulase polysaccharide chains. The second, exocellulases, cleaves 2-4 units from the ends of the exposed chains produced by endocellulas, resulting in the tetrasaccharides or disaccharide such as celloboise. The third, cellobiases, or beta-glucosidase, hydrolyses the endocellulase product into individual monosaccharides. Preferably, a cellulase is 40 percent cellobiase and 60 percent endocellulase.

Pectinases are an enzyme that breaks down pectin, a polysaccharide found in plant cell walls. Commonly referred to as pectic enzymes, they include pectolyases, pectozymes and polygalacturonases. One of the most widely used commercial pectinases is polygalacturonase. It is useful because pectin is the jelly-like matrix which helps cement plant cells together and in which other cell wall components, such as cellulose fibrils, are embedded. Therefore pectinase enzymes are commonly used in processes involving the degradation of plant materials, such as speeding up the extraction of fruit juice from fruit, including apples and sapota.

Polygalacturonases (including, pectin depolymerases, pectinases, endopolygalacturonases, pectolases, pectin hydrolases, pectin polygalacturonases, endopolygalacturonases, poly-alpha-1,4-galacturonide glycanohydrolases, endogalacturonases, endo-D-galacturonases, and poly-glycanohydrolases) are enzymes produced in plants which are involved in the ripening process. Polygalacturonases degrade polygalacturonan present in the cell walls of plants by hydrolysis of the glycosidic bonds that link galacturonic acid residues. Polygalacturonan is a significant carbohydrate component of the pectin network that comprises plant cell walls. Polygalacturonases work to soften the outer walls of biomass. Similarly, phytopathogens use polygalacturonases as a means to weaken the pectin network.

Protease (also termed peptidase or proteinase) is any enzyme that conducts proteolysis, that is, begins protein catabolism by hydrolysis of the peptide bonds that link amino acids together in the polypeptide chain forming the protein. In vascular plants, cellulose is synthesized at the plasma membrane by rosette terminal complexes (RTCs). The RTCs are hexameric protein structures, approximately 25 nanometers in diameter, that contain the cellulose synthase enzymes that synthesize the individual cellulose chains. Each RTC floats in the cell's plasma membrane and "spins" a microfibril into the cell wall. There is therefore a peptide bond at the end of each cellulose fibril and this is the bond that was targeted by the protease. Protease activity refers to the activity of a group of enzymes whose catalytic function is to hydrolyze (breakdown) peptide bonds of proteins.

The one or more enzymes, used alone or in any and all combinations, described above may be used to treat tobacco material which is concurrently or subsequently subjected to a flash drying process. The partial cell wall degradation is about 20 to 60 percent of cellulose (both internal bonds and bonds at the ends) and 20 to 60 percent of the pectin of the tobacco material. Preferably, the partial degradation of the cell walls is 30 to 50 percent of the cellulose (both internal bonds and bonds at the ends) and 30 to 50 percent of the pectin of the tobacco material.

Preferably, the enzyme activity according to the use or the method of the present invention is in the range of 10-500 nanokatals per gram of dried tobacco material (where a katal is the amount of enzyme(s) that convert one mole of dried tobacco material per second).

The enzymes may be employed alone or as enzyme mixtures. The activity of the enzymes is in the range of 10-500 nanokatal per gram dried tobacco material. The enzymes are employed in an aqueous solution, preferably in a pH range between 3.5 and 6.5, preferably between 4 and 6. This is a mildly acidic condition.

The incubation with enzymes preferably takes place between 30 degrees Celsius and 45 degrees Celsius, more preferably between 35 degrees Celsius to 41 degrees Celsius, or most preferably between 38 degrees Celsius to 40 degrees Celsius. The preferred incubation time is function of the effectiveness of the enzyme and its type of activity. Preferrably, the ratio ranges from 125 nanokatals per gram per hour to 2.5 nanokatals per gram per hour. The tobacco enzyme mixture is usually incubated for a period of 1 to 20 hours, preferably 2 to 16 hours, more preferably 2 to 4 hours.

In a further preferred embodiment, the tobacco material is treated with one or more enzymes as specified above and consequently subject to a drying process. Preferably, one of the drying processes used is flash drying, also known as flash tower drying.

In a further preferred embodiment, the tobacco material is treated with one or more enzymes as specified above and in parallel subject to a drying process. Preferably, one of the drying processes used is flash drying, also known as flash tower drying.

The flash tower drying process (or flash drying process) is the conventional flash tower drying process and involves drying with hot air, super-heated steam, or a combination of the two, preferably super-heated steam. Flash tower drying is one of the known processing procedures for increasing the filling power of cut tobacco material. Older models of flash dryers work with hot air. In modern flash dryers super-heated steam is used. The tobacco passes through a pipe with super-heated steam which dries the tobacco. The rapid heat transfer leads to an increase of filling power of the tobacco material due to an opening effect to the tobacco fibres. The cell wall structure of the tobacco material is, however, not affected by the flash tower drying process.

In the drying process according to the present invention, a method gas may be employed which is preferably super-heated steam, such that its heat transfer capability can be improved. The method gas may comprise super-heated water steam. Further provided is the use of one or more cellulose degrading enzymes for enhancing the filling power of tobacco material in a flash tower drying process.

Enzyme treatments were carried out by spraying the enzymes evenly on the tobacco material. Treatments were carried out at 34 percent moisture content wet basis (equivalent to 66 percent dry weight basis). Enzymes were mixed with deionized water prior to spraying. During spraying, tobacco was gently mixed to ensure even dispersion of enzyme on the samples in a rotary drum (rotating cylinder). After enzyme addition tobacco was incubated at a temperature of 40 degrees Celcius in a jacketed rotary drum (heating of the drum through jacket).

Also provided is an apparatus of the present invention which is suitable for performing the method of treating tobacco material to achieve increased filling power as set forth above. The apparatus may comprise two or more vessels, for example a first vessel for conducting steps a) and b) of the method of the present invention as set forth above and a second vessel for conducting step c) of the method of the present invention as set forth above. Typical vessels employed for conducting steps a) or b) are made of glass, metal or a polymer-containing material.

The second vessel may be a conventional dryer such as a rotary dryer, a flash dryer, or a vibrating dryer. The second vessel may contain a heating unit or a heater. The vessels of the apparatus of the present invention may be part of a single process line and may be preferably comprised in one housing.

The subject matter as provided by the present invention is the result of the unexpected finding by the present inventors that cellulose degrading enzymes are a useful, efficient, and effective tool for enhancing filling power in tobacco material. It was also surprisingly found by the present invention that the dry ice expanded tobacco process can be replaced by the above method without a significant loss of filling power of the tobacco material, thereby saving manufacturing costs, capital expenditures, and increasing efficiency.

Preferably, the tobacco material to be dried has a water or moisture content that is not less than about 7 to 8 weight percent of water. More preferably, the moisture content in the tobacco is from about 13 to about 30 weight percent water. Further, by adjusting the properties of the method gas or cooling medium, in particular the content of steam, the moisture content of the tobacco can be controlled.

In particular, the subjecting of the material to hot method gas and the lowering of the temperature of the method gas are conducted in adjacent portions of a pipe in which the method gas flows. The conveying of the material during the expansion and cooling allows to quickly change the temperature around the material and thus to subject the material to the predetermined temperatures in a reliable manner.

The cooling medium may preferably be a cooling gas, such as air. The cooling medium may also preferably be water or water steam. More preferably, the cooling medium is demineralized water or demineralized water steam. Alternatively, or additionally, the cooling medium comprises or is composed of nitrogen, carbon dioxide or Argon. All of these gases are generally not chemically reacting with starch containing products and are therefore not changing the taste or appearance of the product in an undesired manner.

In particular, the method medium or the cooling medium or the method gas and cooling medium comprise less than about ten percent of air, or less than about two percent of oxygen. This prevents the material from being subject to oxidation. Preferably, the cooling medium or method gas is comprised of mainly nitrogen and carbon dioxide. The cooling medium may be injected at several locations, which are in a distance to each other in the downstream direction of the flow of method gas.

In particular, further heat can be applied by the heater, such that the method gas becomes super-heated steam. The steam may in particular replace the gas or air which is introduced in the system together with the tobacco. Therefore, some of the tail gas may be removed from the circulation of method gas before expansion medium is injected into the method gas.

In particular, the heater is arranged upstream the product inlet. The product inlet may be arranged in the high temperature zone. In particular, the heater heats the method gas to about 160 to 600 degrees Celsius, preferably to about 200 degrees Celsius. Therefore, the heater is heated to a temperature of about 220 to 1000 degrees Celsius.

In one embodiment, a cut filler of tobacco obtained by partially degrading the cell walls of tobacco material, the method of obtaining the cut filler of tobacco comprising the steps of:
a) contacting tobacco material using an aqueous solution of one or more enzymes capable of degrading cellulose;
b) incubating the tobacco material with the aqueous solution of one of more enzymes for a period of 1 to 20 hours;
c) drying the tobacco material treated with the one or more enzymes.

The tobacco material is, in particular, cut filler tobacco. However, the tobacco material may also be full or cut tobacco leaves. Cut filler may be used for final products such as smoking articles, in particular cigarettes or cigars, as well as loose tobacco such as roll-your-own and make-your-own tobaccos. Furthermore, the tobacco product may be a tobacco containing product for a smoking device which only heats, but not burns, the tobacco. In particular, the tobacco product differs from expanded tobacco products in the prior art by having a higher expansion level compared to products not treated according to the invention. The tobacco material used in the present invention is selected from stem, strip, midribs, cut filler or reconstituted tobacco, either individually or in any combination thereof. The tobacco material may be uncured tobacco, cured tobacco, whole leaf tobacco or tobacco lamina. Furthermore, the invention provides a tobacco product comprising tobacco processed by the methods, uses or apparatus according to the invention as specified herein.

In one embodiment, the present invention provides a method of partially degrading the cells walls of tobacco material, the method comprising the steps of:
a) contacting the tobacco material using an aqueous solution of one or more enzymes capable of degrading cellulose;
b) incubating the tobacco material with the aqueous solution of one of more enzymes for a period of 1 to 20 hours; and
c) drying the tobacco material treated with the one or more enzymes.

The enzymes employed in this method are as characterized above.

In a preferred embodiment, the method includes a drying step which is a flash tower drying step. The flash tower drying involves drying with hot air and/or super-heated steam. The tobacco material may be dried in the flash tower drying step in 5 to 240 seconds, preferably 15 to 180 seconds or more preferably 10 to 15 seconds. Preferably, the flash tower drying dries the tobacco using a method gas at a temperature between 150 degrees Celsius and 210 degrees Celsius. More preferably the temperature used by the flash tower dryer is 170 degrees Celsius to 190 degrees Celsius.

In the method, one or more enzymes are used in an aqueous solution with a dosage range between 0.23 and 4437 millilitres per kilogram dry weight tobacco material, preferably 0.5-226 millilitres per kilogram dry weight tobacco material. The enzyme activity may be in the range between 10 and 500 nanokatal per gram dry weight tobacco material.

The filling power of tobacco material according to the embodiment of the present invention is enhanced compared to the filling power when using flash tower drying alone. Accordingly, as another embodiment of the present invention the use of one or more cellulose degrading enzymes for enhancing the filling power of tobacco material in a flash tower drying process is provided.

The filling power achieved by using the one or more cellulose degrading enzymes with or without an additional flash tower drying process is preferably comparable to the filling power achieved in conventional industrial processes such as the dry ice expanded tobacco process.

Preferably, the filling power is higher than 4.7 cubic centimeters per gram dry weight tobacco material. More preferably, the filling power is at least 4.9 cubic centimeters per gram dry weight tobacco material.

Preferred enzymes or enzyme compositions of the present invention are set forth in example 1 below and include commercial examples such as Ecopulp R® (an endoclucanase), Corolase 7089® (a protease) and Depol 40L® (a cellulase made up of endoglucanase, cellobiohydrolase, and pectinase). The dosage range as useful within the present invention comprises an enzyme activity range between 10 and 500 nanokatal per gram dry weight tobacco material. The dosage ranges are preferably between 0.23 and 4437 millilitres per kilogram.
Figure 1 shows an illustrative but not limiting effect of the use of enzymatic action according to the invention in the treatment of tobacco material. The tobacco cells applying enzymatic action lose mechanical constraints due to the enzymatic treatment as a partial degradation of cell walls (1 a). In a flash tower drying process the enzyme-treated tobacco material is expanded due to cellular enlarging (1b).
Figure 2 is a microscopic picture showing the illustrative effect of a pectinase on cellulose. The cross-section of tobacco leaf blade and the palisade parenchyma cells are shown. Staining is done with toluidine blue.
Figure 3 is a microscopic picture showing the effect of endoglucanase II on cellulose. A cross-section of the tobacco leaf blade and the palisade parenchyma cells is shown. Staining is done with toluidine blue.

Both figures, Figure 2 and Figure 3 show the partial degradation of the walls of tobacco leaf cells and the increased average cell size as a consequence thereof.

Figure 4 shows the result of the determination of the filling power according to example 1. Filling Power is the ability of tobacco to form a firm cigarette rod at a given moisture content. A high filling power indicates that a lower weight of tobacco is required to produce a cigarette rod than is required with tobacco of lower filling power. The tobacco material used for the tests was cut filler. Some of the experiments resulted in less filling power than the reference water because the cell wall degradation was excessive and lead to a collapse of the internal structure.

Enzyme compositions of the present invention achieve a higher filling power capacity when applied together with a flash tower drying process according to example 1 as compared to a control in which only the flash tower drying process is used.

The following is an example for illustrative purposes.

### Example 1:

The following example shows increased filling power in centimeters cubed per gram for selected enzymes/enzyme mixtures employed in various concentrations and dosage ranges to conventional tobacco leaves. The tobacco material is contacted with an aqueous enzyme solution and incubated for 18 hours at 40 degrees Celsius.

Thereafter, the treated with the one or more enzymes is dried in a super-heated steam with a method gas of 180 degrees Celsius and a cyclisation rate of 21 kilograms per hour. The drying step takes 180 seconds.

The enzymes are characterized in Table 1 below.

**Table 1**

| **Enzyme(s)** | **Enzymatic activity** | **Dosages (nanokatal per gram dry weight)** | **Dosages (millilitres per kilogram dry weight)** |
|---|---|---|---|
| Endoglucanase | Endoglucanase activity (activity of a group of enzymes whose catalytic function is the hydrolysis of cellulose. Such activity is typically measured on hydroxyethylcelluose (HEC)) | 50 and 500 | 2.8 and 28 |
| Protease | Protease activity (Protease activity refers to the activity of a group of enzymes whose catalytic function is to hydrolyze (breakdown) peptide bonds of proteins.) | 10 and 40 | 56 and 226 |
| Cellulase (endoglucanase, cellobiohydrolase), pectinase | Endoglucanase activity | 10 and 100 | 0.5 and 5 |

The results of the detection as shown in Table 2.

**Table 2**

| Enzyme/Activity/Treatment duration | Flash Drying Cycle | Filling Power [cubic centimeters per gram] |
|---|---|---|
| Corolase7089, 40 nanokatal per gram, 18 hours | Drying super-heated steam, 180 degrees, Celsius 21 kg/h 180s | 5.0 |
| Ecopulp R, 50 nanokatal per gram, 18 hours | Drying super-heated steam, 180 degrees Celsius, 21 kg/h 180s | 4.9 |
| Ecopulp R, 500 nanokatal per gram, 18 hours | Drying super-heated steam, 180 degrees Celsius, 21 kg/h 180s | 4.9 |
| Ref water instead of Enzyme, 18 hours | Drying super-heated steam, 180 degrees Celsius, 21 kg/h 180s | 4.7 |
| Corolase 7089, 10 nanokatal per gram, 18 hours | Drying super-heated steam, 180 degrees Celsius, 21 kg/h 180s | 4.7 |
| Depol 40 L, 10 nanokatal per gram, 18 hours | Drying super-heated steam, 180 degrees Celsius, 21 kg/h 180s | 4.6 |
| Depol 40 L, 100 nanokatal per gram, 18 hours | Drying super-heated steam, 180 degrees Celsius, 21 kg/h 180s | 4.6 |

The results of the determination of the filling power are shown in Figure 4. Some of the experiments resulted in less filling power than the reference water because the cell wall degradation was excessive and lead to a collapse of the internal structure.

## Claims

1. A method of partially degrading the cell walls of tobacco material, the method comprising the steps of
(a) contacting tobacco material using an aqueous solution of one or more enzymes capable of degrading cellulose;
(b) incubating the tobacco material with the aqueous solution of one of more enzymes for a period of 1 to 20 hours;
(c) drying the tobacco material treated with the one or more enzymes.

2. The method of claim 1, wherein the one or more enzymes include endogluconase, cellulase, or protease.

3. The method of any of claims 1 or 2, wherein the drying includes a step of flash tower drying.

4. The method of any of the preceding claims, wherein the flash tower drying involves drying with hot air or super-heated steam.

5. The method of any of the preceding claims, wherein the flash tower drying dries the tobacco using a method gas at a temperature between 150°C and 210°C, preferably at about 180 degrees Celsius.

6. The method of any of the preceding claims, wherein the one or more enzymes are used in a dosage of 0.23 - 4437 millilitres per kilogram dry weight tobacco material.

7. The use of one or more enzymes capable of partially degrading cell walls in tobacco leaves.

8. The use of claim 7, wherein the one or more enzymes are capable of degrading cellulose.

9. The use of claim 7 or 8, wherein the one or more enzymes include endogluconase, cellulase, and protease.

10. The use of any of claim 7-9, wherein the tobacco leaves are treated with one or more enzymes according to claims 8 or 9, and subject to a drying process, preferably a flash tower drying process.

11. An apparatus for conducting the method of partially degrading the cell walls of tobacco material, the method comprising the steps of
(a) contacting tobacco material using an aqueous solution of one or more enzymes capable of degrading cellulose;
(b) incubating the tobacco material with the aqueous solution of one of more enzymes for a period of 1 to 20 hours;
(c) drying the tobacco material treated with the one or more enzymes.

12. The apparatus of claim 11 comprising a first vessel for conducting step a) of contacting tobacco material using an aqueous solution of tobacco enzymes of one or more enzymes capable of degrading cellulose and step b) of incubating the tobacco enzyme mixture for a period of 1 to 20 hours; and a second vessel for drying the treated with the one or more enzymes.

13. The apparatus of claim 11 or 12, wherein the second vessel contains a heater, preferably a heater suitable to achieve temperatures so that the method gas becomes super-heated steam.

14. The apparatus of any of claims 11-13, wherein the first and second vessels are comprised in one housing.

15. A cut filler of tobacco obtained by partially degrading the cell walls of tobacco material, the method of obtaining the cut filler of tobacco comprising the steps of:
(a) contacting tobacco material using an aqueous solution of one or more enzymes capable of degrading cellulose;
(b) incubating the tobacco material with the aqueous solution of one of more enzymes for a period of 1 to 20 hours;
(c) drying the tobacco material treated with the one or more enzymes.
